

## UNITED STATES PATENT OFFICE

2,071,626

LEATHER SUBSTITUTE AND METHOD OF  
MAKING THE SAME

Frank Harris, Sharon, Mass., assignor to Plymouth Rubber Company, Inc., Canton, Mass., a corporation of Massachusetts

No Drawing. Application May 28, 1934, Serial  
No. 727,981

8 Claims. (Cl. 91—68)

This invention relates to materials closely simulating leather in appearance and capable of being used in place of leather for some purposes. Material of this general nature has heretofore been made by napping a fabric and then treating the napped face with an adhesive in the nature of a rubber containing liquid so applied thereto as to saturate the nap, and to so treat the material, as by rolling while under tension, to produce a leather-simulating surface. The napping operation, however, which picks the fibers from the individual strands of fabric acts to materially weaken the fabric and for some uses, as for linings for shoes, which are subjected to severe stresses in the pulling over and lasting operation, such weakening is a serious matter.

The present invention has for an object, therefore, to provide material possessing all of the desirable characteristics of the product made from the napped fabric, but without the weakness produced by the napping operation, and which will also have certain other advantages over prior constructions, such as greater flexibility and resistance to abrasion and being less "pipey" when bent.

In accordance with the present invention, therefore, a woven cloth is taken as the foundation material and to this cloth, with its fibers intact, is applied a coating of suitable adhesive cement such as, preferably, a rubber cement, although other types of cement, such as a nitrocellulose cement or combinations of suitable materials, may be employed. One or both surfaces of the cloth may be so coated. Next flock is applied to the adhesively coated surface of the cloth. This may be shaken on and beaten in in accordance with the usual method of putting on flock, or it may be blown on with an air gun under sufficient air pressure to embed the fibers of the flock well into the adhesive. Such flock fibers are usually shorter than the loosened fibers of a napped fabric. Preferably they are cotton. The cement or adhesive is preferably then allowed to harden. Next the material is placed under tension to loosen the fibers and the flocked surface or surfaces are impregnated when under tension with a suitable surfacing binding material, such, for example, as a rubber-containing solution. For both the initial coating and this saturant, a rubber cement with a volatile solvent, or latex, either natural or artificial, is quite suitable and preferably also, where rubber is used, it may contain a suitable vulcanizing agent, together with accelerators, plasticizers, or other usual rubber-modifying or treating constituents, depending on the char-

acteristics desired in the completed product. The saturating adhesive is preferably pressed into the flocked surface as by passing the material between pressure rollers. The saturating material is then set, as by passing it through a drying chamber, and the sheet material is then subjected to further tension, and passed between pressure rollers to apply facial pressure, and allowed or caused to vulcanize or completely set, or the setting or vulcanization may be effected before the final treatment between the pressure rolls. If desired, the material so formed may be further treated with surfacing agents such as pyroxylin, boiled oils, or the like, which will give the desired surface finish to the final product or will facilitate finishing operations such as embossing or the like, or the material may be otherwise surfaced as may be desired.

Material so formed is much stronger than that formed with a napped foundation fabric, so that lighter cloth may be used for equal strength. It also has a more closely bonded surfacing which is not so easily removed by abrasion as is the sheet material made from the napped fabric, as heretofore described. Likewise it has more body, due to the greater mass of fibers in the flocked surface than in the napped surface. When bent it has a finer surface wrinkling or piping, more closely simulating in this respect the piping or wrinkling of high grade leather than is the case of the material having a napped fabric foundation. It likewise is more flexible than this prior material and is capable of more stretching without damage.

From the foregoing description of the product and a method by which it may be made, it should be evident to those skilled in the art that various changes and modifications may be made without departing from the spirit or scope of this invention as defined by the appended claims.

I claim:

1. The method of making a leather substitute, which comprises adhesively applying flock to the surface of a woven cloth fabric, applying a binding saturant to said flocked surface, and subjecting said material to facial pressure while under tension.
2. The method of making a leather substitute, which comprises applying an adhesive to the surface of a woven cloth fabric, applying flock to said adhesive and permitting the adhesive to harden, and then applying a binding saturant to said flocked surface while the material is under tension, and applying pressure thereto also while the material is under tension.

3. The method of making a leather substitute, which comprises applying an adhesive to the surface of a woven cloth fabric, applying flock to said adhesive and permitting the adhesive to harden, and then applying a rubber-containing binding agent to said flocked surface while the material is under tension, and applying pressure thereto while the material is under tension.
4. The method of making a leather substitute, which comprises applying an adhesive to the surface of a woven fabric, applying flock to said adhesive and permitting the adhesive to harden and then applying a rubber-containing binding saturant to said flocked surface while the material is under tension, subjecting the material to pressure, drying and setting the saturant, again pressing under tension, and surface-coating the material.
5. The method of making a leather substitute, which comprises applying an adhesive to the surface of a woven cloth fabric, applying flock to said adhesive and permitting the adhesive to harden, and then applying a binding saturant to said flocked surface while the material is under tension, subjecting the material to pressure, dry-
- ing the saturant, and again pressing under tension.
6. The method of making a leather substitute, which comprises applying an adhesive to the surface of a woven cloth fabric, applying flock to said adhesive and permitting the adhesive to harden, and then applying a binding saturant to said flocked surface while the material is under tension, subjecting the material to pressure, drying the saturant, again pressing under tension and surface-coating the material.
7. A leather substitute, which comprises a layer of woven cloth coated with rubber into which is embedded flock, and surfaced with rubber saturating said flock and in compressed condition produced by the process of claim 8.
8. The method which comprises applying an adhesive to the surface of a woven textile fabric, applying flock thereto and allowing the adhesive to harden to bond the flock to the fabric, then while the material is under tension saturating the flocked surface with a rubber-containing solution, setting and finishing the surface to simulate leather.

FRANK HARRIS. 25